# EUROPEAN PATENT SPECIFICATION

(11) **EP 0 007 198 B1**
(45) Date of publication and mention of the grant of the patent: **04.08.1982**
(21) Application number: 79301238.6
(22) Date of filing: 26.06.1979
(51) Int. Cl.: F24C 3/10, F24C 5/14, F23Q 7/00, H05B 3/10

(54) **Igniter**
Zündvorrichtung
Dispositif d'allumage

(30) Priority: 29.06.1978 GB 2835778
(43) Date of publication of application: 23.01.1980
(73) Proprietor: MORGANITE ELECTROHEAT LIMITED, Perth, Scotland (GB)
(72) Inventor: Bryce, Lawrence Miller, Nunthorpe Middleborough, Cleveland (GB); Roebuck, Peter Hamish Athey, Perthshire, Scotland (GB)
(74) Representative: Farwell, William Robert

## Description

### Field of the invention

The invention relates to fuel-ignition in heating boilers or other domestic or industrial gas or oil fuelled appliances.

### Background

We have sought alternatives to the electronic and piezoelectric spark ignition systems now widely used in gas cookers, domestic central heating boilers and similar gas equipment, and to resistance-heated rod igniters that have been proposed but not to our knowledge used, at least in the United Kingdom. Our aim has been an igniter that is not unduly position sensitive in equipment so that design and layout are not restricted, that allows an energy input sufficiently high to give positive and reliable ignition with natural gas, that works at voltages and powers safe and easily provided by inexpensive means, and that is easily serviced by gas and heating fitters. We have also sought to meet the standard requirement that ignition times of 2 to 5 seconds and preferably 3 seconds or less shall be attainable, and also that in domestic equipment a power rating of 10 watts or less at suitable voltages such as the standard 24 volts for many control units shall be used. Rod igniters of silicon carbide cannot meet these requirements, being used at mains voltage with high power requirements, and any attempt to scale down the conventional ceramic techniques by which they are made gives bodies that are too fragile to use.

In DE-A1-2 501 894 is disclosed a fuel-ignition device comprising an electrically conductive carbide heating element and means for passing a heating current to the element to raise it to fuel-ignition temperature. Further, the use of other ceramic materials as heating elements is known, (DE-B-1 238 126).

None of the prior art proposals meet the difficult task of simultaneously satisfying the criteria we have given above, for gas ignition primarily but also for oil.

### The present invention

We however have found successful a fuel-ignition device comprising an electrically conductive carbide, boride, silicide, nitride, oxide or other ceramic monofilament as a heating element and means for passing a heating current to the filament to raise it to fuel-ignition temperature.

The filaments on which the success of the invention depends are made for example, by vapour deposition onto a preformed core or by drawing from a melt, and show a high tensile strength, up to 340 Kg/mm² in one particular silicon carbide filament we have tested. Such strengths may be contrasted with typical strengths below 10 Kg/mm² for ceramic bodies made by conventional ceramic techniques such as extrusion of plastic mixes, pressing, tamping and the like, whether or not followed by final machining stages.

To provide for ready conduction of current in the cold, and guard against a surge of current as the filament warms up from ambient temperature, the filament has a more conductive core of carbon or of tungsten or other metal. A carbon core is preferred, on which for example silicon carbide, the preferred ceramic, is readily vapour deposited.

Silicon carbide filaments are produced for example for reinforcement purposes in composite materials, and one particular filament that is suitable for the present purpose is produced by continuous vapour deposition of A-silicon carbide on a carbon filament core, final diameter 140 microns. Such a filament is strong enough to stand repeated thermal cycling from room temperature to over 1100°C in ignition, as well as mechanical shocks to which equipment may be subjected.

The carbon core is important to the functioning of the device. At low temperatures, the carbon core itself carries the bulk of the current due to the relatively high cold resistance of the surrounding silicon carbide. Similar solid or tungsten-core silicon carbide filaments require increased power compared to the carbon core filament to attain ignition temperature due to their higher cold resistances. Power requirements can be controlled by varying the filament diameter and in particular the cross-sectional ratio of carbon core to silicon carbide annulus.

In the installed device it is desirable for short ignition times that a continuous pre- heating current should be passed through the filament, when for example it is readily provided that the filament shall reach the ignition temperature in five seconds or less on passage of the heating current. The presence of a conductive core is desirable for passage of such a current, which for example may be 20-30 mA at 10-15 V in the particular 140 micron carbon core silicon carbide filament described above. A suitable preheating current for given circumstances is readily found by experiment, though the filament temperature it corresponds to is not easily measured.

Ignition temperatures, readily measured by pyrometer observations, vary according to the conditions but sample figures for stoichiometric mixtures with air are:

A suitable nominal filament temperature for ignition, as measured by the final filament temperature under a given power in still air, is readily established for given conditions of fuel/air flow, uniformity of mixing and temperature. It cannot be less than the ignition temperatures quoted above and for practical conditions is likely to be 1000°C or above and in any event not less than 800° or 900°C.

The mounting of the filament is preferably in a tubular or other disposable holder for impingement of a fuel/air flow on the filament. Preferably further the filament is retained in place by a crimped mounting of copper or other metal freely conductive of heat and electricity.

### Detailed discussion

In the following detailed discussion the filament is referred to as 'fibre'.

Initial tests were conducted by replacing the piezo-electric igniter of a natural gas cooker by a 15 mm length 21 of the 140 micron diameter fibre, clamped by simple terminal screws in a holder 22 and placed 30 mm from the gas orifice 23, across the path of the gas jet. The arrangement is shown in Fig. 1 of the accompanying drawings, the old igniter 24 - being used as the gas source.

The terminals were then connected in a test circuit with a mains transformer (50 cycles), a voltmeter and an ammeter and a current of 250 mA at 40 volts applied. The fibre heated to 1180°C and gave ignition in less than a second.

In a similar test a fibre 1 cm long was used and gave satisfactory ignition at 24 volts. This fibre was then cycled repeatedly from room temperature to 1150°C, one second on and one second off. There was no treatment of the fibre ends to improve contact, but even under this simple test the fibre underwent 6360 cycles before failure, which occurred at the contacts.

A further 1 cm sample of the fibre was then tested for resistance at different temperatures. The resistance dropped from 260 ohms at 600°C (the lowest temperature used) to 155 ohms at 800°C and 140 ohms at 1000°C, and levelled off at 110 ohms at 1300⁰C, giving a valuable protection against overheating but a temperature sufficient to secure ignition in all reasonable circumstances (see Fig. 2). The cold resistance was 435 ohms.

This graph differs from that of β-SiC due to the role played by the carbon core.

In a second test application shown in Fig. 3 of the accompanying drawings, the igniter fibre itself is fitted in a small holder rather like a domestic fuse and equally easily replaceable. The holder consists of a ceramic tube 1 with opposed holes 2 for gas flow, and terminal caps 5 with solder connections 3 for the fibre 4. The holder is clipped at 7 into copper mountings 6 to which current supply wires 8 are fixed. Gas is directed onto the fibre by a burner nozzle 9 fed from a supply pipe 10 through a solenoid operated valve 11, the supply wires 12 of which are also shown.

To avoid any problems of melting of the solder at the terminals, other forms of terminal connections were also tested, in particular brazing, noble metal cements and mechanical fixing. Of these, the most satisfactory was crimping of the fibre into a copper capillary tube of outside diameter 1.46 mm and inside diameter 0.33-4.43 mm.

The copper tube was soldered into the fuse housing and tested using the same apparatus as described in Fig. 3.

Wherr the already heated fibre igniter is introduced into the natural gas flame, the temperature of the fibre increases by up to 200°C. Though this should theoretically enhance oxidation, and reduce the service life, it appears that the natural gas shroud about the igniter actually forms a protective barrier against oxidation.

In all the early tests, the emphasis was on thermal shock testing through rapid cycling. Though the fibre igniter itself has low thermal mass and as such dissipated most of its heat within the short 'off periods of cycling, some residual heat was maintained, particularly by the surrounding connections and hence the igniter was not allowed to reach ambient temperature and hence its true high value of cold resistance. In a typical working environment, however, where say for a domestic gas cooker the igniter would be subjected to use only about a dozen times a day, it would be allowed to reach room temperature i.e. attain its original high cold resistance.

Cycling on this basis (30 minutes to 1 hour off period) showed a time delay prior to ignition (a slow power build up to overcome the cold resistance). The time delay, in the range 5 to 20 seconds, is undesirable but is readily overcome by applying a constant low power current of for example 0.5 watt to maintain the temperature above ambient, e.g. at 200°C.

In practical application of the invention to a cooker one igniter in the centre of the hob can light a small auxiliary burner and flame tubes then light the main burners as required. A separate igniter is used for the oven.

## Claims

1_{:} A fuel-ignition device comprising an electrically conductive carbide, boride, silicide, nitride, oxide or other ceramic heating element and means for passing a heating current to the element to raise it to fuel-ignition temperature, characterised in that the element is a monofilament with a tungsten or other metal, or carbon, core on which the ceramic has been formed by vapour deposition or otherwise and which is of higher electrical conductivity than the ceramic.

2. A device according to Claim 1, in which the ceramic is silicon carbide.

3. A device according to Claims 1 or 2 wherein the filament is mounted in tubular or other disposable holder for impingement of a fuevair flow on the filament.

4. A device according to any preceding claim, wherein the filament is retained in place by a crimped mounting of copper or other conductive metal.

5. A device according to any preceding claim, further having means for passing a continuous pre-heating current to the filament to allow it to reach the ignition temperature in five seconds or less on passage of the heating current.

6. A heating boiler or other domestic or industrial gas or oil fuelled appliance fitted with an ignition device according to any preceding claim.

## Revendications

1. Dispositif d'allumage de combustible comprenant un élément céramique de chauffage conducteur de l'électricité en carbure, borure, siliciure, nitrure, oxyde, ou autre, et des moyens pour faire passer un courant de chauffage dans l'élément pour élever sa température à celle l'allumage du combustible, caractérisé en ce que l'élément est un monofilament à noyau en tungstène ou autre métal, ou en carbone, sur lequel la céramique a été formée par dépôt par vaporisation, ou autrement, et qui a une conductivité électrique plus élevée que la céramique.

2. Dispositif selon la revendication 1, caractérisé en ce que le céramique est du carbure de silicium.

3. Dispositif selon la revendication 1 ou la revendication 2, caractérisé en ce que le filament est monté dans un support démontable tubulaire ou autre, pour qu'un flux de mélange combustible/air frappe le filament.

4. Dispositif selon l'une quelconque des revendications précédentes, caractérisé en ce que le filament est maintenu en place par une monture sertie en cuivre ou en un autre métal conducteur.

5. Dispositif selon l'une quelconque des revendications précédentes, caractérisé en ce qu'il comprend en outre des moyens pour faire passer un courant de préchauffage continu dans le filament pour lui permettre d'atteindre la température d'allumage en 5 secondes ou moins lors du passage du courant de chauffage.

6. Chaudière de chauffage ou autre appareil domestique ou industriel à gaz ou à mazout équipée d'un dispositif d'allumage selon l'une quelconque des revendications précédentes.

## Patentansprüche

1. Vorrichtung zum Zünden von gasförmigem oder flüssigem Brennstoff mit einem Heizelement aus elektrisch leitendem Material wie Carbid, Borid, Silizid, Nitrit, Oxid oder einem anderen Oxid-Keramik-Material sowie mit Mitteln (6, 7, 8; 22) für die Zufuhr von Strom an das Heizelement, durch den dieses auf die Brennstoff-Zündtemperatur erhitzt wird, dadurch gekennzeichnet, daß das Heizelement ein Heizfaden (21; 4) ist, der einen Kern aus Wolfram oder einem anderen Metall bzw. aus Kohlenstoff aufweist, auf den das Oxid-Keramik-Material durch Aufdampfen oder anderweitig aufgebracht ist und der eine höhere elektrische Leitfähigkeit als das Oxid-Keramik-Material aufweist.

2. Vorrichtung nach Anspruch 1, dadurch gekennzeichnet, daß das Oxid-Keramik-Material Siliziumcarbid ist.

3. Vorrichtung nach Anspruch 1 oder 2, dadurch gekennzeichnet, daß der Heizfaden (4) in einer zum Beispiel rohrförmigen Wegwerfhalterung (1,5) befestigt ist, in der er einem Brennstoff-Luftgemisch-Strom ausgesetzt werden kann.

4. Vorrichtung nacn einem der vorhergehenden Ansprüche, dadurch gekennzeichnet, daß der Heizfaden von aus Kupfer oder einem anderen metallischen Leitermaterial bestehenden gequetschten Elementen gehalten wird.

5. Vorrichtung nach einem der vorhergehenden Ansprüche, gekennzeichnet durch Mittel, durch die dauernd ein Vorheizstrom zugeführt wird, so daß der Heizfaden bei Zufuhr des eigentlichen Heizstroms die Zündtemperatur nach höchstens 5 Sekunden erreicht.

6. Vorrichtung nach einem der vorhergehenden Ansprüche, dadurch gekennzeichnet, daß sie bei einem Warmwasserbereiter oder einem anderen in Haushalt oder Industrie verwendeten gas- oder ölgefeuertem Gerät eingesetzt ist.
